

# UNITED STATES PATENT OFFICE.

ARTHUR MÜLLER, OF FÜRSTENWALDE-ON-THE-SPREE, GERMANY, ASSIGNOR TO THE FIRM  
OF G. P. DROSSBACH & CO., OF FREIBERG, GERMANY.

## PROCESS OF MANUFACTURING INCANDESCENT MANTLES.

No. 927,374.

Specification of Letters Patent.

Patented July 6, 1909.

Application filed October 4, 1907. Serial No. 395,895.

*To all whom it may concern:*

Be it known that I, ARTHUR MÜLLER, a subject of the Emperor of Austria-Hungary, residing at Fürstenwalde-on-the-Spree, in the 5 Kingdom of Prussia and Empire of Germany, have invented a new and useful Improvement in the Manufacture of Incandescent Mantles, of which the following is a specification.

10 My invention relates to improvements in the manufacture of incandescent mantles, and its object is to impregnate the fabric of the latter with colloidal solutions of the oxidhydrates of rare earths for the purpose hereinafter set forth.

In the manufacture of incandescent mantles the fabrics have hitherto always been saturated with crystalloidal solutions of salts (nitrates) of the rare earths employed which 20 on reduction of the fabric to ash by heating to incandescence leave the corresponding oxids. According to my new process, on the contrary, the fibers of any suitable nature, such, for instance, as vegetable fibers (cotton, 25 linen, ramie) or artificial silk, are impregnated with a colloidal solution of the oxidhydrates, the latter being absorbed direct and retained. In the prior process the solution of the salts used is merely mechanically 30 absorbed, so that the salts only adhere superficially to the fiber and can be wholly removed by boiling in water. According to my invention, on the other hand, there is formed, as in the dyeing process, an insoluble, 35 firmly adhering absorption-combination between the steeped fiber-substance and the colloidal oxid-hydrates. The great advantage of this method over the prior process is that by a single impregnation, without any 40 subsequent treatment of the fibers, the earths are most intimately incorporated, adhering firmly and uniformly.

If an incandescent mantle impregnated according to the ordinary method and not 45 burned off, is immersed in water, the salts are rapidly and completely extracted from the fabric. If, however, a mantle impregnated with colloidal solution and not burned off is put in water, the fabric still retains 50 considerable quantities of the impregnated earths.

The colloidal solution of thorium hydrate can be prepared in various ways. (1). According to well-known methods: acting upon

the solid oxid with mineral acids, or dialyses 55 of dilute thorium nitrate solution toward pure water. (2). A simple manner of preparing colloidal thorium hydroxid solution is based upon the resolution (peptisation) of freshly precipitated gelatinous thorium oxid 60 by means of small quantities of added thorium nitrate. For instance, from 100 grains of dry thorium nitrate the thorium hydroxid is precipitated by means of an alkali, the gelatinous precipitate then carefully washed 65 on the filter to remove entirely the excess of the alkali and the salts, and the pure precipitate then distributed in a little water and heated to boiling point. Hereupon an aqueous solution of 10.2 grams of dry thorium 70 nitrate is added in small quantities and the liquid kept boiling. After about half an hour the thorium hydroxid will have been converted into a clear, slightly bluish opalescent colloidal solution. That this solution is 75 actually colloidal can be readily determined by its behavoir toward precipitants: small quantities of alkali, and of mineral acids, immediately throw down the colloidal dissolved thorium hydroxid as an insoluble 80 gelatinous precipitate. To the colloidal solution so obtained the necessary quantity of cerium nitrate is added and the solution then diluted for use, depending upon the desired degree of concentration of the impregnating 85 fluid. All the remaining operations in the manufacture of the incandescent mantle can be conducted as ordinarily.

Having thus described my invention, what I claim as new is:

1. In the manufacture of incandescent mantles, in impregnating the fabric of the latter with a colloidal solution of an oxidhydrate of a rare earth, substantially as described.

2. In the manufacture of incandescent mantles, in impregnating the fabric of the latter with a fluid containing a colloidal solution of an oxid-hydrate of a rare earth, substantially as described.

In testimony whereof I have signed my name to this specification in the presence of two subscribing witnesses.

ARTHUR MÜLLER.

Witnesses:

PAUL ARRON,  
CLARE SIMON.